# EUROPEAN PATENT SPECIFICATION

(11) **EP 0 526 942 B1**
(45) Date of publication and mention of the grant of the patent: **10.04.1996**
(21) Application number: 92202329.6
(22) Date of filing: 28.07.1992
(51) Int. Cl.: C10M 169/04, C21D 1/58

(54) **Liquid composition**
Flüssige Zusammensetzung
Composition liquide

(30) Priority: 30.07.1991 GB 9116382
(43) Date of publication of application: 10.02.1993
(73) Proprietor: SHELL INTERNATIONALE RESEARCH MAATSCHAPPIJ B.V., NL-2596 HR Den Haag (NL)
(72) Inventor: Muijs, Herman Mathieu, NL-1031 CM Amsterdam (NL); Beers, Nicolaas Cornelis Maria, NL-1031 CM Amsterdam (NL); Wiersma, Rendert Jan, NL-1031 CM Amsterdam (NL)

(56) References cited:
- EP-A- 0 025 328
- EP-A- 0 178 354
- EP-A- 0 354 621
- EP-A- 0 413 374
- DE-A- 2 411 827
- DE-A- 3 742 572
- GB-A- 2 081 299
- GB-A- 2 232 665
- US-A- 4 140 642
- US-A- 4 164 474

## Description

The invention relates to a liquid composition and to a process for the preparation of such a liquid composition. The invention specifically relates to a liquid composition comprising
a) an alkylated xylenesulphonic acid salt:
b) a glycol having a molecular weight of between 200 and 1500;
c) an aromatic, paraffinic or naphthenic oil; and
d) less than 1 percent by weight of water, calculated on the total composition.

From European patent EP-A-0 413374 is known a composition comprising an alkylated xylenesulphonic acid salt and a glycol having a molecular weight of between 200 and 1500, suitable for enhancing recovery of oil from a subterranean oil-containing reservoir.

The composition according to the invention, however, is an oil-containing clear and liquid solution of an alkylated xylenesulphonic acid salt, which is substantially anhydrous as herein defined. The composition has an excellent storage stability and a suitable viscosity. It may be used as a protective fluid in metal-working industry. It may also be used as a quenching oil in metal processing. It shows no phase separation nor crystallization at zero degree C.

Preferred compositions are those wherein an alkylated xylenesulphonic acid salt is an ortho-xylenesulphonic acid salt of the formula wherein M is an alkali metal or ammonium and A is a C₈-C₃₀ alkyl group, preferably a C₁₂-C₂₀ alkyl group.

The long chain-alkyl group is bound to the aromatic ring from its 2-position to its mid-position.

Preferably the glycol is polyethylene glycol or polypropylene glycol. Preferred molecular weights range from 200 to 1200, more preferred from 300 to 1000.

Preferred compositions comprise 50 to 65 percent by weight of alkylated xylenesulphonic acid salt; 5 to 20 percent by weight of glycol; less than one percent by weight of water and the balance being an oil, preferably a naphthenic oil or paraffinic oil.

The compositions according to the invention may be prepared by neutralizing an alkylated xylenesulphonic acid in the presence of an aromatic, paraffinic or naphthenic oil, subsequently adding a glycol to the neutralized reaction mixture and distilling off the water to a level of less than one percent by weight. The distillation is carried out at a temperature of 80 °C to 100 °C.

Of special importance in the compositions according to the invention are the C₁₃, C₁₄-alkyl ortho-xylene sulphonic acid salt and the C₁₆-, C₁₈-alkyl ortho-xylene sulphonic acid salt, specifically the sodium salt.

It is possible to prepare alkyl ortho-xylene sulphonates in a concentration of about 60 percent by weight of active material in an oil, containing also less than 10 percent by weight of water (without a glycol). Said composition is generally a rigid gel and with only containing water in a small range of 4.2 to 4.8 percent by weight, the composition is liquid. Low water content formulations of this type (without glycol) are generally solids.

For preparing liquid formulations the water content is replaced by polyglycol. After the glycol has been added to the formulation, the water is distilled off. This process may be facilitated by introducing in the neutralization vessel nitrogen or air.

### Example 1

610 g of alkylated ortho-xylene sulphonic acids having the chemical structure wherein A represents C₁₆- and C₁₈-alkyl (average mol. weight 425) were neutralized with 124.6 g of aqueous 47% by weight of sodium hydroxide solution in 257.7 g of paraffinic oil.

The formulation comprised 60% by weight of active matter, 10% by weight of water and had a kinematic viscosity of 340 mm/s at 60 °c and a solidification point of 30 °C to 40 °c.

Subsequently 95 g of polyethylene glycol (average mol. weight 300) was admixed with the neutralized formulation and the temperature was raised to 95 °C in order to remove the water by stripping. Stripping was continued until 87.4 g of water was removed.

The water content was 0.6 percent by weight on the total composition of 1000 g. This product had a kinematic viscosity of 1780 mm/s at 60 °C, and remained a liquid even below 0 °C without crystallization.

### Example 2

609.2 g of alkylated ortho-xylene sulphonic acids having the chemical structure wherein A is C₁₃- and C₁₄-alkyl (average mol. weight 380) were neutralized with 134.8 g of aqueous 47% by weight of sodium hydroxide solution in 256.0 g of paraffinic oil. This formulation had a kinematic viscosity of 190 mm/s and a solidification point of 30 °C to 40 °C.

Subsequently 95 g of polyethylene glycol (average mol. weight 300) was admixed with the neutralized formulation and the temperature was raised to 95 °C to remove the water by stripping. Stripping was continued until 95 g of water was removed.

The water content was 0.5 percent by weight on the total composition of 1000 g. This product had a kinematic viscosity of 4950 mm/s, and remained a liquid even at 0 °C.

### Example 3

The process of Example 1 was repeated, whereby instead of a paraffinic oil a naphthenic oil was used. The amounts of the components were the same as those used in the process of Example 1.

Subsequently 95 g of polyethylene glycol with an average mol. weight of 1000 was admixed with the neutralized formulation and the temperature was raised to 95 °C to remove the water by stripping. Stripping was continued until 87.4 g of water was removed.

The water content was 0.6 percent by weight on the total composition of 1000 g. This product was just yet a liquid at 0 °C without any crystallization.

The naphthenic oil had the following properties:

| | |
|---|---|
| kinematic viscosity at 100 °C | 2.28 mm/s |
| flash point | >148 °C |
| pour point | -39 °C or below |

The paraffinic oil had the following properties:

| | |
|---|---|
| kinematic viscosity at 100 °C | 4.4 -4.9 mm/s |
| flash point | >200 °C |
| pour point | -18 °C or below |

## Claims

1. A liquid composition in the form of a solution comprising
a) an alkylated xylenesulphonic acid salt;
b) a glycol having a molecular weight of between 200 and 1500;
c) an aromatic, paraffinic or naphthenic oil; and
d) less than 1 percent by weight of water, calculated on the total composition.

2. A composition as claimed in claim 1, wherein is used an ortho-xylene sulphonic acid salt of the formula wherein M is an alkali metal or ammonium and A is a C₈-C₃₀ alkyl group.

3. A composition as claimed in claim 2, wherein the alkyl group is a C₁₂-C₂₀ alkyl group.

4. A composition as claimed in claims 1-3, wherein polyethylene glycol having an average molecular weight between 200 and 1000 is used.

5. A composition as claimed in claims 1-4, wherein 50 to 65 percent by weight of alkylated xylenesulphonic acid salt; 5 to 20 percent by weight of glycol; less than 1 percent by weight of water and 14 to 44 percent by weight of the oil are present.

6. A process for the preparation of a composition as claimed in claim 1 which comprises neutralizing an alkylated xylenesulphonic acid in the presence of an aromatic, paraffinic or naphthenic oil to the alkylated xylenesulphonic acid salt and water; subsequently adding a glycol to the neutralized reaction mixture and distilling off the water to a level of less than 1 percent by weight.

7. A process as claimed in claim 6 wherein the distillation takes place at a temperature of 80 °C to 100 °C.

## Patentansprüche

1. Flüssige Zusammensetzung in Form einer Lösung, enthaltend
a) ein alkyliertes Xylolsulfonsäuresalz,
b) ein Glykol mit einem Molekulargewicht von 200 bis 1500,
c) ein aromatisches, paraffinisches oder naphthenisches Öl und
d) weniger als 1 Gew.-% Wasser, bezogen auf die Gesamtzusammensetzung.

2. Zusammensetzung nach Anspruch 1, in der ein ortho-Xylolsulfonsäuresalz der Formel verwendet wird, worin M für ein Alkalimetall oder Ammonium und A für eine C₈-C₃₀-Alkylgruppe stehen.

3. Zusammensetzung nach Anspruch 2, in der es sich bei der Alkylgruppe um eine C₁₂-C₂₀-Alkylgruppe handelt.

4. Zusammensetzung nach den Ansprüchen 1-3, in der man Polyethylenglykol mit einem mittleren Molekulargewicht von 200 bis 1000 verwendet.

5. Zusammensetzung nach den Ansprüchen 1-4, in der 50 bis 65 Gew.-% eines alkylierten Xylolsulfonsäuresalzes, 5 bis 20 Gew.-% eines Glykols, weniger als 1 Gew.-% Wasser und 14 bis 44 Gew.-% des Öls vorliegen.

6. Verfahren zur Herstellung einer Zusammensetzung nach Anspruch 1, bei dem man eine alkylierte Xylolsulfonsäure in Gegenwart eines aromatischen, paraffinischen oder naphthenischen Öls zu dem alkylierten Xylolsulfonsäuresalz und Wasser neutralisiert, anschließend der neutralisierten Reaktionsmischung ein Glykol zufügt und das Wasser bis zu einem Gehalt von weniger als 1 Gew.-% abdestilliert.

7. Verfahren nach Anspruch 6, bei dem man die Destillation bei einer Temperatur von 80°C bis 100°C durchführt.

## Revendications

1. Composition liquide sous forme d'une solution, comprenant:
a) un sel d'acide xylènesulfonique alkylé;
b) un glycol ayant une masse moléculaire comprise entre 200 et 1 500;
c) une huile aromatique, paraffinique ou naphténique et,
d) moins de 1% en poids d'eau, par rapport à la composition totale.

2. Composition selon la revendication 1, dans laquelle on utilise un sel d'acide ortho-xylènesulfonique de formule dans laquelle M est un métal alcalin ou un ammonium et A est un groupe alkyle en C₈-C₃₀.

3. Composition selon la revendication 2, dans laquelle le groupe alkyle est un groupe alkyle en C₁₂-C₂₀.

4. Composition selon les revendications 1-3, dans laquelle on utilise un polyéthylèneglycol ayant une masse moléculaire moyenne comprise entre 200 et 1 000.

5. Composition selon les revendications 1-4, dans laquelle sont présents 50 à 65% en poids de sel d'acides xylènesulfoniques alkylés; 5 à 20% en poids de glycol; moins de 1% en poids d'eau et 14 à 44% en poids de l'huile.

6. Procédé de préparation d'une composition selon la revendication 1, qui comprend la neutralisation d'un acide xylènesulfonique alkylé en présence d'une huile aromatique, paraffinique ou naphténique, en sel d'acide xylènesulfonique alkylé et eau, ensuite l'addition d'un glycol au mélange réactionnel neutralisé et l'élimination de l'eau par distillation jusqu'à une proportion inférieure à 1% en poids.

7. Procédé selon la revendication 6, dans lequel la distillation a lieu à une température de 80°C à 100°C.
